

Jan. 5, 1943.

E. H. VOIGTMAN ET AL

2,307,342

SELF MOLDING COUNTER

Filed May 5, 1941

2 Sheets-Sheet 1

Fig. 1.



Fig. 2.



Fig. 3.



Fig. 4.



Fig. 5.



INVENTORS:

Edward H. Voigtmann

Harry B. Kettell

BY Scans, Pond & Anderson

Atty's

Jan. 5, 1943.

E. H. VOIGTMAN ET AL

2,307,342

SELF MOLDING COUNTER

Filed May 5, 1941

2 Sheets-Sheet 2

Fig. 6.



Fig. 8.

Fig. 7.



Fig. 9.



INVENTOR

Edward H. Voigtman  
BY Harry B. Kellogg  
Soans, Pond & Anderson  
Atty's

## UNITED STATES PATENT OFFICE

2,307,342

## SELF-MOLDING COUNTER

Edward H. Voigtman and Harry B. Kellogg, Neenah, Wis., assignors to Paper Patents Company, a corporation of Wisconsin

Application May 5, 1941, Serial No. 391,830

5 Claims. (Cl. 36—68)

This invention relates to shoe stiffeners, particularly counters and to an improved method of installing and lasting the same.

Heretofore, it has been the general practice in the shoe making industry to utilize two general types of counters. In the better grade shoes it has been customary to use leather counters which are worked wet and are lasted to exact size. This procedure, however, involves an expensive raw material; it requires that the counter blanks be conditioned or mulled in an atmosphere of 100% relative humidity for periods of from 24 to 72 hours; and it necessitates a long drying period usually of from three to five days on the last. The procedure is, therefore, not only time consuming, but it requires a very large number of lasts with accompanying difficulties and expense in handling and storage during manufacture.

In the cheaper grades of shoes, it is common practice to use what are known as pre-molded counters. These counters are usually manufactured of a laminated material which can be molded to size by the use of heat and pressure. The counters are made prior to the shoe manufacturing operation, and are installed during the lasting of the shoe. This procedure permits very substantial reduction in the lasting time, usually from a matter of days to a matter of hours, but because it is economically impractical to maintain stocks of counters for more than a few of the many widths, in any given size, only a small percentage of preformed counters will fit the last perfectly. Hence, insofar as fit is concerned, the preformed counters are very inferior to the leather counters, also the need for maintaining large stocks of counters in order to obtain even approximate fits, is highly undesirable from the viewpoint of the manufacturer.

The principal object of the present invention is to overcome these disadvantages of the prior art counters by providing a counter having normal physical properties similar to leather counters and the capability of being molded to size during the lasting operation, but which can be dried or otherwise restored to its normal stiff condition in a much shorter interval of time than is possible with leather counters. In addition, it is desired to provide an improved counter in accordance with the above stated principal object and which shall be reasonably inexpensive to manufacture which shall be capable of long and satisfactory wear when installed in a shoe.

As will hereinafter appear, these objects are accomplished by the provision of an improved, composite counter and method of installing the

same. These will be made more apparent by reference to the accompanying drawings and the following description of certain preferred embodiments of the invention.

5 In the drawings:

Fig. 1 is a perspective view of a sheet of laminated material particularly designed for manufacturing counters or other stiffeners in accordance with the present invention;

10 Fig. 2 is a plan view of a counter blank which has been cut from a sheet of the laminated material illustrated in Fig. 1;

Fig. 3 is a plan view showing the blank of Fig. 1 following the skiving operation;

15 Fig. 4 is sectional view on line 4—4 of Fig. 3;

Fig. 5 is a diagrammatic view illustrating one step in the installation of counters in accordance with the present invention;

20 Fig. 6 is a perspective view of a shoe equipped with counter and toe cap stiffeners in accordance with the present invention;

Fig. 7 is an enlarged sectional view on line 7—7 of Fig. 6 and illustrates the relation of the counter to the other parts of the shoe; and

25 Figs. 8 and 9 are perspective views, similar to Figs. 2 and 3, of a toe cap stiffener blank before and after skiving.

The composite sheet material illustrated in Fig. 1 is preferably of two ply laminated construction. The inner ply or sheet A, which serves as the backing ply, is preferably a thin, flexible, water-resistant material, having physical characteristics closely resembling those of leather. The outer ply or sheet B, which serves as the stiffening ply, is a considerably stiffer sheet than the inner ply A. During the lasting operation it is necessary to temporarily soften at least the stiff ply B. To make this possible, that ply is manufactured by impregnating a base fiber with a stiffening compound, which also acts as the primary binder for the base fiber, and with a secondary binder which is relatively flexible and which is resistant to agents which soften the primary binder or stiffening agent. The two plies or sheets A and B are permanently fastened together by an adhesive such as rubber latex, which will not lose its strength during the subsequent counter forming operations.

In a particularly satisfactory embodiment of the invention, the flexible backing ply A consists of a sheet of artificial leather which is made by superposing from about 20 to 40 sheets of thin, creped, cellulosic tissue having a basis weight within the range of from about 4 to 9 pounds for 480 sheets 24 x 36 inches, impregnating the super-

posed sheets with rubber (latex), and then pressing and heat treating the product as described in United States Letters Patent to Sewal No. 1,915,339, to produce a sheet approximately .020 to .055 inch thick and having a weight of from 1.45 to .80 pounds per square yard, the total rubber (latex) content amounting to from about 28 to 37% of the dry weight of the sheet. It will be understood, however, that other artificial leather materials or similar products can be used. The flexible ply A should, however, have a thickness within the range of about .020 to .055 inch and should be sufficiently flexible to permit easy lasting without prior softening.

In this same embodiment of the invention, the sheet B is normally quite stiff and is made by superposing from about 50 to 70 sheets of thin, creped, cellulosic tissue having a basis weight within the range of from 4 to 9 pounds for 480 sheets 24 x 36 inches, impregnating the superposed sheets with a mixture of latex and raw starch, pressing and heat treating the impregnated product to coagulate the latex and gelatinize the starch in situ. The completed sheet has a thickness within the range of about .075 to .115 inch and has a weight of from about 2 to 3 pounds per square yard. The stiffness of this sheet can be varied by varying the starch content. Low percentages of starch (2 to 5% of the dry weight of the sheet) yield fairly flexible sheets, and high percentages of starch (7 to 14% of the dry weight of the sheet) yield very stiff sheets. The rubber content should be held within from 11 to 26% of the total weight of the dry sheet. The very best results were obtained when the starch content was about 8% of the total weight of the dry sheet and the rubber content was about 16% of the total weight of the dry sheet.

In the manufacture of this embodiment of the invention, the flexible backing sheet A and the stiffening sheet B are laminated together, with the adhesive in between, and then calendered. The calendering reduces the thickness of the composite sheet from about 5 to 20%. As a result, in this embodiment of the invention, the flexible backing sheet A after calendering has a thickness within the range of from about .016 to .052 inch, and the stiffening sheet B has a thickness within the range of from about .060 to .110 inch.

Various other sheet materials may be used for the stiff ply B. However, at least a substantial portion of this ply should include the following three constituents: (1) a fibrous base, which may consist of superposed sheets of thin, cellulosic tissue, water or air-laid fibrous felts, or even a thick fabric capable of impregnation, (2) a primary binder or stiffening agent which may consist of starch casein, resins or other materials capable of losing their stiffness when soaked in a suitable solvent, preferably a solvent which includes water and an organic solvent, and (3) a secondary binder capable of holding the sheet together when the primary binder has been softened, i. e. the secondary binder must not be soluble in the same solvents which soften the primary binder. Latex, artificial rubber, synthetic resins, and other material are satisfactory for this purpose.

As will hereinafter appear, the best results are obtained when the sheet plies A and B constitute multiply impregnated products such as have been described above, and particularly satisfactory results are obtained when the stiff ply employs starch and latex as the primary and secondary binders respectively. As will hereinafter appear,

the starch-latex impregnated sheet can be readily softened by the use of an inexpensive easy to use softening agent—such as a mixture of water and alcohol—and counters made from this material will dry on the last in a reasonably short time.

In the manufacture and use of counters or other stiffeners made from the above described materials, a counter blank such as is illustrated at 11 in Fig. 2 is cut from the laminated sheet. The edge of the blank 11 is then skived as illustrated at 13 so as to expose an edge portion of the flexible backing ply A. This provides a flexible edge in the finished shoe while preserving the desired stiffness in the counter. If the stiff ply is of the starch-latex type, the skived blank is then soaked in a warm solution (about 100° F.) of water and alcohol, water and acetone, or water, alcohol, and acetone for from about 10 to 15 minutes, as illustrated in Fig. 5. Either ethyl or methyl alcohol can be used with water, in substantially equal proportions by volume. If acetone is used, the proportion should be about from 45 to 55 parts of acetone to from 55 to 45 parts of water, by volume. If the alcohol water-acetone mixture is used, best results are obtained with the latex starch sheet material by using 50% water, 40% ethyl alcohol and 10% acetone, by volume. Other proportions can be used. Ordinarily, it will be found undesirable to use more than about 65% or less than about 25% of the organic solvent or solvents. If desired, the counters can be rendered highly water resistant as an incident to the softening operation. To accomplish this, it is necessary merely to add a paraffin wax emulsion or similar water-proofing agent to the softening agent and when this is done, the water-proofing material will be deposited on the surface of the counter in a uniform film as the softening agent dries.

If the stiff ply utilizes a stiffening agent other than starch, or if an entirely different material is employed for the stiff layer, other solvents may be indicated. It will be understood, however, that the material used for softening the stiff layer must not soften the secondary binder; if it does the blank will fall apart.

After 10 to 15 minutes submergence in the softening material, the blanks 11 will be quite limp and each can be inserted between the quarter lining 17 and the outer stock 19 of a shoe, as illustrated in Fig. 6. The shoe can then be built around the last in the usual manner. On drying, which in the case of the starch latex material should not require more than 3 or 4 hours, the counter will be found to have assumed the exact shape and size of the last, and will possess physical properties closely approximating those of leather counters. However, the time consuming mulling and drying on-the-last operations, which are a necessary incident to the manufacture of leather counters, are eliminated with resultant very considerable economies in the manufacturing cost of the shoes without any loss of quality.

The novel material described in the foregoing can, of course, be utilized in the manufacture of toe caps, and suitable blanks, as cut and as skived, are illustrated in Figs. 8 and 9 at 21 and 23. The position of the toe cap in the shoe is illustrated in outline by the dotted lines 25 in Fig. 6 similar to the counter.

As stated previously, the preferred material utilizes a multiply latex or rubber impregnated sheet for the flexible backing ply A and a multiply latex (or rubber) starch impregnated sheet for the stiff ply B, with a latex adhesive for perma-

nently joining the two plies. This combination permits the use of relatively inexpensive mixtures of alcohol and water as the softening agent. At the same time it produces a counter which is very easy to handle during the lasting operation, and which will possess substantially the same physical characteristics as leather in the finished shoe. Various modifications in the sheet product and in the procedure described in the foregoing will suggest themselves to those skilled in the art. It is desired, therefore, that the accompanying claims shall be accorded the broadest reasonable construction consistent with the language appearing therein and the prior art.

We claim as our invention:

1. A multiply shoe stiffener comprising a backing ply of felted and compacted cellulosic fibers held together by a binder which contains rubber in sufficient amounts to cause said ply to possess substantially the same physical characteristics of high flexibility and resilience as leather, and a stiffening ply permanently secured to said backing ply, said stiffening ply being normally much stiffer than said backing ply and being formed of felted and compacted cellulosic fibers held together by a cooked starch, primary binder, which serves to stiffen said ply and which can be softened by mixtures of water and organic solvents, and by a rubber, secondary binder which is substantially unaffected by the mixtures of water and organic solvents used to soften said primary binder.

2. A multiply shoe stiffener comprising a backing ply which has a thickness within the range of from about .016 to .052 inch and which comprises fibrous material held together by a binder which contains rubber in sufficient amounts to cause said ply to possess substantially the same physical characteristics of high flexibility and resilience as leather, and a stiffening ply permanently secured to said backing ply, said stiffening ply being normally stiffer than said backing ply, having a thickness within the range of from about .060 to .110 inch and comprising a fibrous base, a cooked starch, primary binder, and a rubber secondary binder which is present in greater amounts by weight than said primary binder, said starch primary binder constituting from about 2 to 14 percent of the dry weight of said stiffening ply, and said rubber secondary binder constituting from about 11 to 26 per cent of the dry weight of said stiffening ply.

3. A multiply shoe stiffener comprising a backing ply having substantially the same physical characteristics as leather, said backing ply having a thickness of within the range of from about .016 to .052 inch and comprising a fibrous base and a rubber binder which constitutes from about

- 5 28 to 37 percent of the dry weight of said ply, and a stiffening ply permanently secured to said backing ply, said stiffening ply being normally stiffer than said backing ply, having a thickness within the range of from about .060 to .110 inch and comprising compacted cellulosic fibers, a cooked starch, primary binder impregnating said fibers, and a rubber, secondary binder also impregnating said fibers and being present in greater amounts by weight than said primary binder, said starch primary binder constituting from about 2 to 14 percent of the dry weight of said stiffening ply and said rubber, secondary binder constituting from about 11 to 26 percent of the dry weight of said stiffening ply.
- 10 15 4. A multiply shoe stiffener comprising a backing ply of fibrous material held together by a flexible binder in such amounts that said ply possesses substantially the same physical characteristics of high flexibility and resilience as leather, and a stiffening ply permanently secured to said backing ply, said stiffening ply being normally much stiffer than said backing ply and comprising a fibrous base held together by a cooked starch, primary binder, which serves to stiffen said ply and which can be temporarily softened by suitable solvents, and by a rubber secondary binder which is present in greater amounts by weight than said primary binder, said starch primary binder constituting from 2 to 14% of the dry weight of said stiffening ply and said rubber secondary binder constituting from 11 to 26% of the dry weight of said stiffening ply.
- 20 25 30 35 40 45 50 55 5. A multiply shoe stiffener comprising a backing ply of felted and compacted cellulosic fibers held together by a binder which contains rubber in sufficient amounts to cause said ply to possess substantially the same physical characteristics of high flexibility and resilience as leather, and a stiffening ply permanently secured to said backing ply, said stiffening ply being normally much stiffer than said backing ply and being formed of felted and compacted cellulosic fibers held together by a cooked starch, primary binder, which serves to stiffen said ply and which can be softened by mixtures of water and organic solvents, and by a rubber, secondary binder which is present in greater amounts by weight than said primary binder, said starch primary binder constituting from 2 to 14 per cent of the dry weight of said stiffening ply, and said rubber secondary binder constituting from 11 to 26 per cent of the dry weight of said stiffening ply.

EDWARD H. VOIGTMAN.  
HARRY B. KELLOGG.